

Jan. 8, 1946.

G. S. DE KADT

2,392,582

TREATMENT OF WET SPUN PROTEIN PRODUCTS

Filed Feb. 19, 1941



Inventor:  
G. S. DE KADT

By *Alfredo S. C. C. C.*  
Attorney.

## UNITED STATES PATENT OFFICE

2,392,582

## TREATMENT OF WET SPUN PROTEIN PRODUCTS

George Stephan de Kadt, Leeuwarden, Netherlands; vested in the Alien Property Custodian

Application February 19, 1941, Serial No. 379,672  
In the Netherlands December 27, 1939

7 Claims. (Cl. 18—54)

This invention relates to a process for treating with water vapor or steam products such as fibers, filaments, threads, bands, films and the like which are obtained by the extrusion into a coagulating bath, of a protein solution particularly solutions prepared with the aid of alkali from casein and other globular proteins.

In my copending application Serial No. 257,029 I have described a process for minimizing the tendency to shrinkage of artificial fibres, threads and the like obtained by extrusion into a coagulating bath, of a protein solution, which has been prepared with the aid of alkali. According to that process the products are subjected to the action of steam or water vapor, if desired, in admixture with other vapors or gases, before the products are introduced into a hardening bath. By that process a considerable improvement of the mechanical properties of these products is obtained. It seems that this result is due to the fact that by the treatment with water vapor, water condenses on the products, but I do not wish to be limited to any definite theory for the explanation of the phenomenon.

It is the object of my present invention to provide an improved and effective method for carrying out this treatment with water vapor of the products obtained by extrusion into a coagulating bath of protein solutions, particularly solutions of casein and other globular proteins, which have been prepared with the aid of alkali.

Another object of my invention is the provision of a method of treating the extruded products under such conditions that the certainty of successful operation and improved results are assured.

Another object of my invention is to provide a method whereby improved results are obtained by a uniform and compensating treatment of the extruded products with diluted spinning bath.

Other objects and advantages of my invention will be apparent as it is better understood by reference to the specification and accompanying drawing, which illustrates diagrammatically an embodiment adapted for practice of my invention, it being understood that my invention is not limited to the details hereafter set forth or shown in the drawing.

I have found that the above mentioned treatment with steam or water vapor can be carried out in a particularly advantageous manner by causing the water vapor to act on the products while they are moving over at least one vertically arranged pair of horizontal rollers. If desired, the steam or water vapor may be mixed with other vaporous or gaseous substances influencing the properties of the products, for example those having a hardening action, such as for instance ammonia, methanol, sulfur dioxide, alcohol, carbon dioxide, etc.

In carrying out my invention, I prefer to immerse the bottom roller in a bath, for it has been found that there drops down from the rollers a spinning bath residue diluted by condensed water vapor and having an acid concentration of approximately two thirds of that of the spinning bath. For example, in using a spinning bath containing 6% of acetic acid and 20% of sodium sulfate the first bath residue dropping down from the rollers contains approximately 4% of acetic acid and 16% of sodium sulfate. The layer of spinning bath diluted by the condensation of the water vapor surrounds the thread bundles and exerts a uniform and compensating influence, which is not the case with a horizontal arrangement of the pairs of rollers, which causes formation of drops and accumulation of liquid at the bottom side of the thread bundles.

As I have described in my copending application Serial No. 257,029 the steam or water vapor may be made to act on the products by directing a steam jet onto the products, but the rollers over which the products are passed according to my present invention may also be arranged in a room in which a damp and more or less warm atmosphere prevails, which is preferably obtained by blowing steam into the room. It is not necessary to obtain a high temperature by means of the water vapor since the favorable action is effected even at a temperature as low as approximately 40° C.

I have further found that a uniform impregnation of the thread with the diluted spinning bath can be obtained in a still better manner by immersing the bottom roller in the diluted spinning bath. It will be obvious that in carrying out the treatment with water vapor on a number of pairs of rollers the acid and salt concentration decreases gradually.

In treating the freshly spun threads care has to be taken that by the action of the water vapor and the condensation caused thereby the decrease of the salt concentration is not too great, because in that case the threads will swell again. On the other hand it is of importance to remove as much as possible residual spinning bath, particularly the acid, in order not to contaminate the hardening baths. For this purpose a salt solution, such as one containing sodium sulfate in an amount of approximately 10-15% can be used as a bath in which the rollers revolve.

I have found that the presence of some methanol is not objectionable, so that according to my invention from an economical viewpoint use of the spent hardening bath which apart from salt, approximately 10 to 15% salt, still contains 0.1 to 0.3% of methanol is even preferable.

According to my invention it is also possible, however, to use the washing water with which the liquids of the hardening baths are washed

from the threads. In some cases it is desirable to dissolve first a small amount of salt in this washing water, since it is desirable that its salt content corresponds to that of the hardening baths, which in the case of sodium sulfate contain about 10% of salt. Obviously, however, also other salts and other quantities may be used.

In the drawing:

Fig. 1 is a diagrammatic side view of an embodiment for carrying out the process according to the invention;

Fig. 2 is a diagrammatic side view of a pair of rollers with another arrangement of the steaming device;

Fig. 3 is a diagrammatic side view of a pair of rollers comprising a bottom roller revolving in a bath;

Fig. 4 is a diagrammatic front view of a pair of rollers around which the threads are conducted several times;

Fig. 5 is a diagrammatic side view of a curling device comprising a profiled top roller of the pair of rollers, which cooperates with a profiled third roller;

Fig. 6 is a diagrammatic side view of a curling device comprising a profiled top roller of the pair of rollers, which cooperates with a third rubber roller;

Fig. 7 is a diagrammatic front view of a pair of conical rollers for stretching the thread; and

Fig. 8 is a diagrammatic front view of a pair of stepped rollers for stretching the thread.

According to Fig. 1 the protein solution is extruded into spinning paths 1 through series of spinnerettes 2, the single thread bundles being drawn away by drawing rollers 4. The combined thread bundles 5 are passed over vertically arranged pairs of horizontal rollers 6 and the liquid dripping from the threads and the rollers is collected in baths 7. From the perforated tube 8 arranged between the two pairs of rollers steam is blown onto the moving threads which are conducted over a dosing roller 9 to a cutting device not shown.

Fig. 2 illustrates how the steam pipe 8 may be arranged between the rollers of one pair and Fig. 3 shows the embodiment in which the bottom roller 6 revolves in the bath 7'.

In order to avoid a large number of pairs of rollers the threads may be wound around the rollers several times, which embodiment is illustrated by Fig. 4 in which the numerals indicate the same parts as in the Figures 1-3. In this case the threads may be separated with the aid of thread guides or other means.

According to my invention the products can be fixed in a curled condition by carrying out the treatment with steam simultaneously with a curling treatment, for instance by means of a curling device comprising at least one profile roller. This may be carried out by using as top roller of the pair a profile roller cooperating with a third roller. Fig. 5 shows how the top roller 6 of a pair of rollers is a profiled roller cooperating with an additional profiled roller 12. A thread 5 passes between the rollers 6 and 12 is treated with steam from the pipe 8. Fig. 6 shows a similar curling device consisting of the profiled top roller 6 of the pair of rollers, which cooperates with a rubber roller 13 pressing the thread 5, while steam is supplied by the pipe 8.

If during the treatment with water vapour

some tension is maintained, the thread is stretched because by its plasticity and a kind of flow process is caused by the tension. This flow process in the thread may in this manner be used for stretching the thread, whereby not only its strength is increased, but especially longer threads are spun. By using a number of pairs of rollers this stretching can be carried out best by giving every subsequent pair of rollers a higher speed than the preceding pair. In using a limited number of pairs of rollers the same result can be obtained by application of conical or staged rollers. Fig. 7 shows how the thread is passed several times around a pair of conical rollers 10 and Fig. 8 illustrates how the same result may be obtained by using stepped rollers 11.

Various changes may be made in the details disclosed in the foregoing specification without departing from the invention or sacrificing the advantages thereof.

I claim:

1. The process which comprises extruding an alkaline protein solution into a coagulating bath; thereupon conducting the extruded product through a path comprising substantially vertical portions; and subjecting the said product, as it is conducted through the said path, to the action of an atmosphere which is at least 40° C. and substantially saturated with water vapor.

2. The process which comprises extruding an alkaline protein solution into a coagulating bath, thereupon conducting the extruded product through a path comprising substantially vertical portions; and blowing steam onto said product as it is conducted through the said path.

3. The process which comprises extruding an alkaline protein solution into a coagulating bath; thereupon conducting the extruded product through a path comprising substantially vertical portions; subjecting the said product, as it is conducted downwardly through the said path, to the action of an atmosphere which is at least 40° C. and substantially saturated with water vapor; and immersing the said product in a salt solution at the lowest part of said path.

4. The process which comprises extruding an alkaline protein solution into a coagulating bath; thereupon conducting the extruded product through a path comprising substantially vertical portions; subjecting the said product, as it is conducted downwardly through the said path, to the action of an atmosphere which is at least 40° C. and substantially saturated with water vapor; collecting, at the lowest part of said path, drippings from said product along said substantially vertical portions; and immersing the said product in said collected drippings at the lowest part of said path.

5. The process as defined in claim 1 in which methanal is mixed with the water vapor while the product is conducted through a path comprising substantially vertical portions.

6. The process as defined in claim 1 in which sulfur dioxide is mixed with the water vapor while the product is conducted through a path comprising substantially vertical portions.

7. The process as defined in claim 1 in which alcohol is mixed with the water vapor while the product is conducted through a path comprising substantially vertical portions.

GEORGE STEPHAN DE KADT.